

March 18, 1952

L. R. KOLLER ET AL

2,590,018

PRODUCTION OF COLORED IMAGES

Filed Oct. 24, 1950

2 SHEETS—SHEET 1



Inventors:  
Lewis R. Koller,  
Ferd E. Williams,  
by *Paul A. Frank*  
Their Attorney.

March 18, 1952

L. R. KOLLER ET AL

2,590,018

PRODUCTION OF COLORED IMAGES

Filed Oct. 24, 1950

2 SHEETS—SHEET 2



Inventors:  
Lewis R. Koller,  
Ferd E. Williams,  
by *Paul A. Frank*  
Their Attorney.

## UNITED STATES PATENT OFFICE

2,590,018

## PRODUCTION OF COLORED IMAGES

Lewis R. Koller and Ferd E. Williams, Schenectady, N. Y., assignors to General Electric Company, a corporation of New York

Application October 24, 1950, Serial No. 191,862

13 Claims. (Cl. 313—92)

1

This invention relates to the production of colored images as in color television, color radar and the like. More particularly, it relates to a cathode ray tube for producing color effects and to the colored light producing screen employed therein.

It has been proposed heretofore to provide in a colored image producing cathode ray tube a screen comprising a plurality of superimposed layers of different colored light producing phosphors and to regulate the potential of the exciting electron beam so that only the desired phosphor layer is excited to produce a particular color. This system of selective excitation of phosphor layers, as in any arrangement of superimposed layers of electron energy absorbing materials, is based upon the fact that the potential of an electron beam may be adjusted to allow the electrons to penetrate to a certain depth in the media before giving up a substantial part of their energy, which in the case of phosphors is manifested in a light effect.

In order to provide a continuous phosphor layer by the usual methods of deposition, such as by allowing the particles to settle from a liquid suspension, layers are produced which are a number of particles thick. It has been found that in the system of such layers so formed, in order to present a continuous phosphor surface to the electron barrage, the electron voltages or potentials required to penetrate to the farthest layer to produce the desired range of colors are excessively high and above those normally desirable in a commercial or home television receiver or in radar apparatus. The production of such high potentials also requires more equipment and a larger power supply. There is, further, a large amount of absorption and scattering of light between the particles in such gross screens which detracts from the brightness and resolution of colors produced.

Attempts have been made to produce thinner screens in order to lower the requisite electron potentials. As a practical matter, if screens are of such reduced thickness as to require electron potentials of reasonably low intensity, there are also voids between the particles of phosphor material through which electrons may pass without producing any luminescence or light in the particular layer. There is, consequently, no absorption of electron energy and light production at those particular points in the layer, the electron beam proceeding unhindered to the next layer where an undesired color or one not corresponding to the beam signal voltage, is pro-

duced. The net result is that a fluorescent screen made up of layers having voids does not give a faithful reproduction of the subject scanned in that it produces colors other than those natural to the subject.

An object of this invention is to produce an improved colored image producing screen.

Another object is to provide a colored image producing screen in which the colored image is characterized by increased brightness.

A further object of the invention is to provide such a screen which will operate at relatively lower electron beam exciting potentials than heretofore.

15 15 A still further object is to provide such a screen which has enhanced voltage-brightness characteristics.

Another object of the present invention is to provide such a screen which provides increased 20 sharpness of color separation.

Another object is to produce such a screen in which the image is reproduced in purer colors.

Another object of the invention is to provide 25 such a screen which will faithfully reproduce the true colors of an object.

A further object is to provide a cathode ray tube for accomplishing the above objects.

A still further object of the invention is to provide a colored image system for the realization 30 of the above objects.

Other objects will become apparent and the invention better understood from a consideration of the following description and the drawing in which Fig. 1 shows a cross-section of a 35 portion of the colored image producing screen of the present invention; Fig. 2a is a plot of brightness versus electron beam voltage for a gross liquid-settled three color screen; Fig. 2b is a similar plot for a flotation type screen of the 40 present invention; Fig. 2c is a similar plot for a flotation type three color screen of the present invention having between the layers thereof electron absorbing barriers; Fig. 3 is a spectrogram plot of such a screen at three different electron beam potentials illustrating the purity of colors obtainable using the present invention; and Fig. 4 shows a typical circuit in connection with which the present screen may be employed.

50 It has been found that an improved colored image producing cathode ray tube screen may be readily produced.

It has further been found that an improved cathode ray tube screen for the production of 55 colored images may be made by providing a plu-

rality of mono-particle thick layers of different colored light producing luminescent materials or phosphors, the thickness of each layer being such that the maximum excitation is obtained with the electron beam to which it is sensitive. Preferably, the layers are separated by light transparent, electrically non-conductive barriers which are capable of absorbing electron energy.

The principle upon which this invention is based is that the penetration of electrons emitted from any source, such as an electron gun in a cathode ray tube, depends upon their velocity which varies as the square of their potential. With a given material to be penetrated, the higher the impinging velocity or potential, the greater is the electron penetration. It is also known that an electron beam gives up most of its energy at a particular depth in the material. If, then, three layers of phosphors, each of which produces a different colored light upon excitation, are superimposed one upon the other to form a composite screen, a potential or voltage may be applied to electrons impinging on the screen to cause them to penetrate to any desired depth and then give up most of their energy. Depending upon the initial velocity or potential, this may be made to occur in the first, or succeeding layer and the light produced is mainly the color of the light produced by the phosphor layer in which most of the energy of the electron beam is lost with some color from other layers in which energy is absorbed. Thus, if all the energy from an electron beam is absorbed in a first, red light producing layer, the color emitted is red. If the beam is adjusted to penetrate to and lose most of its energy in a second blue light producing phosphor layer, the color is mainly blue with some red, depending on how much of the energy is absorbed in the first, red layer. Similarly, if the electron beam is adjusted to lose most of its energy in a third, green light producing phosphor layer, the resultant color is mainly green. The amount of red and blue color depends again on the energy absorbed in the first and second layers.

It is obvious that in order to obtain similar brightness response to the electron beam throughout the expanse of any one phosphor layer, the layer should be of uniform thickness. At the same time it should be continuous and thin enough to enable selective excitation by electron beams of low intensity.

A method of making such phosphor coatings is described in copending application Serial No. 172,449, filed July 7, 1950, by Lewis R. Koller and assigned to the same assignee as the present application, the teaching of the above-cited application being included by reference in this application. In the above application it is taught that continuous, mono-particle thick continuous layers of powders, including phosphors, may be placed on a base structure by forming a mono-particle thick layer of the powder on a liquid, passing the surface to be coated upward through the layer and drying. It is further taught that successive mono-particle layers may be produced by simply drying each preceding layer before adding another by the same method.

The use of continuous, thin phosphor layers one particle thick permits the excitation of a particle phosphor layer at substantially lower electron beam potentials than in the case of gross layers since the screen may be made of small particles which absorb just enough electron energy to give a maximum light effect and no more. This is in contrast to ordinary continuous screens in which

the excessive thickness of the layers necessitates very high values of electron energy. In general, the overall absorption of electron energy by mono-particle thick layers is about one-third that of ordinary multi-particle thick screens. At the same time the mono-particle thick layer deposited, as taught herein, affords a maximum coverage of the area upon which it is deposited. This is to be distinguished from thin layers deposited by ordinary methods which have an excessive number of voids or gaps.

Representative examples of transparent screen materials which may be used in connection with the present invention are as follows. Typical red colored light producing phosphors, which may be used, among others, are zinc-cadmium sulphide, magnesium silicate, magnesium germinate, and magnesium phosphate; typical blue phosphors are zinc sulphide and calcium magnesium silicate, while typical green phosphors are willemite or zinc orthosilicate and magnesium aluminate. Using mono-particle thick layers of red, blue, and green phosphors which are, respectively, 2.8 microns, 6.1 microns, and 19.3 microns thick the layers may be excited by electron beams of 10 kilovolts, 18 kilovolts, and 32 kilovolts in that order. When the red, blue, and green layers are  $0.5\mu$ ,  $4.1\mu$ , and  $29\mu$  thick they are excited by electrons having potentials of 6 kilovolts, 12 kilovolts, and 25 kilovolts. As a practical matter, the thickness of the phosphor next to the base of the screen is immaterial so long as it is thick enough to absorb all the energy in any electron beam impinging upon it. In the present instance this is the green phosphor.

Mono-particle thick layers of phosphors are further of great advantage in that their extreme thinness and smoothness makes possible a more abrupt change in color with change in voltage.

While screens made solely of mono-particle thick layers of phosphors have superior colored image producing characteristics, the purity of the colored light produced by any one layer when excited by an electron beam may be enhanced by placing light transparent, electrically non-conductive, electron energy absorbing barriers or layers between the phosphor layers. These layers serve to absorb a certain amount of the energy of the electron beam and may be so adjusted in thickness as to insure that any particular phosphor layer beyond the barrier and farther from the electron beam source is subjected to electrons having a potential with a definite lower voltage or potential limit. In other words, the barriers provide a certain critical voltage below which there is no excitation of the succeeding phosphor layer. While any light transparent, electrically non-conductive electron energy absorbing material may be used for the barriers described herein, finely divided mica and silica are preferred. Alkali silicates may also be employed. These materials are normally applied in the same manner as the phosphors though they may be applied by other means such as, in the case of silica, by the condensation of the vaporized material on the surface to be coated. In a mica layer about 4.0 microns thick the energy loss for 15 kilovolt electrons is about 7.5 kilovolts while for 40 kilovolt electrons the loss is about 2.4 kilovolts. Silica is typically used in thinner layers than mica, down to about  $0.1\mu$  thick. For such a layer the energy absorbed is somewhat less than that lost in the above-mentioned mica layer.

In delimiting a certain critical voltage below which there can be no excitation of a succeed-

ing phosphor layer, the purity of color from each such succeeding layer is enhanced. For example, with successive layers of red, blue, and green light producing phosphors exposed to the electron beam in that order, a barrier between the red and blue layers results in greater purity of the red color at low voltages. As the voltage is raised above the critical value necessary to enable it to pass the first barrier, the brightness of the blue color increases rapidly. The effect of the barrier between the blue and green layers is to permit the attainment of maximum brightness in the blue layer relative to the red layer before there is any excitation of the green layer.

A partial cross-sectional view of a composite screen made up of various mono-particle thick layers is shown in Fig. 1. The composite phosphor screen is laid on glass base 1 which may be flat or have any desired radius of curvature. Preferably, the red, blue, and green light producing phosphors are laid in inverse order on the glass base, that is, the green layer 2 is laid adjacent the base, the blue layer 3 next, and the red layer 4 next. Light transparent, non-conductive or insulating barriers 5 and 6 are preferably placed respectively between the red and blue and blue and green layers. Phosphor layers 3 and 4 are one particle thick and a particle size is selected for each layer which will permit the absorption of the proper amount of the energy of an electron beam to give the desired brightness. Phosphor layer 2 need not be a mono-particle thick layer, but may be liquid-settled to a thickness which will preferably absorb all electron energy entering it. Preferably, though not necessarily, an aluminum film 7 is placed over the outermost layer 4 of phosphor. This aluminum film serves to drain off any electrostatic charge which may tend to accumulate on the phosphor screen. It also serves to reflect light which otherwise would be diverted to the interior of the cathode ray tube of which the screen is a part, and reduces halation effects.

The advantages of the present mono-particle phosphor layers, and particularly the present mono-particle layers having electron energy absorbing layers therebetween, over ordinary gross phosphor layers will be made clear by reference to Figs. 2a-2c. In these figures the brightness of various phosphor screens are measured by a photocell using a suitable filter for each color and plotted against the impinging electron beam potential on an oscillograph trace. The screen of Fig. 2a is a three color red, blue, and green phosphor screen with the green phosphor laid next to the glass base by the usual liquid-settling method to a density of 4.5 mg. per  $\text{cm}^2$ , the particles averaging under  $6\mu$  in size, and the blue and red phosphors laid in the same manner successively above it in that order. At electron beam voltages up at 25 kilovolts, as shown in Fig. 2a, only the red phosphor emitted any color. No color trace was visible for the blue or green phosphors.

The screen of Fig. 2b was laid down in the same order as in Fig. 2a. However, only the green phosphor was formed by liquid-settling means to a density of 4.5 mg. per  $\text{cm}^2$  for particles averaging less than  $6\mu$  in size. The blue and red phosphor layers were laid down by the flotation method mentioned elsewhere herein and consisted of substantially continuous, mono-particle thick layers of particles averaging less than  $6\mu$  in size. The advantage of the mono-particle thick layers over the gross layers of Fig.

2a will at once be seen. Whereas in the gross layers of Fig. 2a, at voltages less than 25 kilovolts only the red phosphor emitted any color, in the mono-particle layer screen of Fig. 2b, at 13 kilovolts the blue phosphor emitted a color which was about 56 per cent as bright as the red color. Likewise, at 13 kilovolts the brightness of the green phosphor emission was about 29 per cent that of the red. This means that for the present mono-particle phosphor layers, the electron beam, at relatively low voltages, penetrates the various phosphor layers to produce varied color effects. This is to be distinguished from the gross layers of Fig. 2a for which at voltages less than 25 kilovolts the electron beam had not penetrated even the first red layer.

Fig. 2c represents similar data for a screen like that of Fig. 2b except that silica barriers about  $1\mu$  thick were placed between the red and blue and the blue and green mono-particle thick phosphor layers. It will be noted that Fig. 2c is quite similar to Fig. 2b in that the electron beam again penetrated to all layers to give a varicolored effect. However, it will also be noted that the effect of the barrier was to displace the oscillograph traces somewhat to the right. Thus, at 13 kilovolts the brightness of the blue color emission was only about 37 per cent of that of the red emission and the brightness of the green color was only 13 per cent of that of the red. As the electron beam potential increased, the preponderance of red decreased being displaced by a blue emission which was increased more rapidly in brightness over the green by means of the barrier. As the potential was still further increased, the green emission likewise increased more rapidly in brightness than when no barrier was present.

It will be appreciated then that the present 40 mono-particle thick multi-layer screen permits the production of a plurality of colors at electron beam potentials under 25 kilovolts whereas the gross layer screens will produce at such voltages only the color of the first layer impinged upon. 45 The presence of electron energy absorbing barriers between the phosphor layers further improves the purity of the colors in that as the electron beam potential increases the preponderance of red emission decreases.

50 Another beneficial effect of the present barriers is that, should voids be present to a very slight extent between phosphor particles, the barrier layers absorb enough electron energy to insure that a false color is not produced. In the absence of the barrier, an electron beam meant to excite a particular layer but which strikes a void space between the configuration of the particles in the mono-particle thick layer proceeds unhindered to the next layer to excite a successive 55 layer not intended to be excited. The result is that regions of one color are interposed with foreign colors which detract from the quality of the image reproduced. When the present barriers are employed, their thickness may be so 60 adjusted that energy is absorbed in them to the extent that the succeeding layer of phosphor is not excited except by a voltage which is enough higher so that undesirable interference of colors is obviated.

65 The extreme sharpness of the color change obtainable using the present mono-particle layers separated by electron-energy absorbing layers is in contrast to that produced by gross superimposed layers of phosphor material. Fig. 3 shows typical results obtained with mono-particle lay-

ers averaging less than  $6\mu$  in size, except for the green phosphor layer, when exposed to electron beams of various potentials, the phosphors being arranged in order with the green color producing material nearest the glass with overlying successive layers of blue and red phosphors. Under 5 kilovolt excitation the energy-wavelength distribution is shown in curve 8, the light coming almost entirely from the red layer to give a pure red color. Curve 9 shows results under 21 kilovolt excitation with the light coming from both the red and blue layer, but predominately from the blue. At 45 kilovolts, as shown in curve 10, the light comes from all three layers, but mostly from the green. This spectral distribution is typical of that obtainable at even lower electron beam potentials as with the screen of Fig. 2c.

The grain size of the phosphors making up the present layers determines the electron beam potentials at which they operate. For example, with red, blue, and green phosphor particle sizes of 2.8, 6.1, and 19.3 microns, respectively, the exciting electrons are 10, 18, and 32 kilovolts in that order. With red, blue, and green mono-particle layers 0.5, 4.1, and 29 microns thick the corresponding electron voltages are 6, 12, and 25. In all cases the silica barriers used between phosphor layers were about two or three microns thick.

As a matter of actual practice the thickness of the layer next to the glass surface is not of importance so long as it blocks the passage of all electrons. While this layer may be of mono-particle structure, it may also be laid down by any of the usual settling processes and is normally of a density of 4.5 mg. per  $\text{cm}^2$ .

Usually the phosphor layers are formed on the glass with the phosphor of the highest efficiency lowermost and the others superimposed thereon in decreasing order of efficiency. In the present examples this order has been green, blue, and red with the electron beam striking the layers in inverse order.

In order that the means of applying the teachings of the present invention may be more readily understood, reference is made to Fig. 4 which shows schematically a color television receiving unit. It will be understood, of course, that this particular arrangement is shown not in a limiting sense, but merely for purposes of illustration. It will also be understood that the present screen may be used wherever it is desired to convert electrical pulses into color; typical examples being radar and television.

Reference is made to Fig. 4 for a typical example of the operation of the present colored image producing fluorescent screen when used in a cathode ray tube as part of a television system which for the most part is shown schematically.

Cathode ray tube 11 has an evacuated envelope 12 containing an electron gun 13, a deflecting system 14, semiconductive coating 15, and screen 16. Electrons emitted by cathode 17 are controlled and focussed by control grid 18, attracted by first anode 19 and further accelerated toward screen 16 by semiconductive coating 15 which acts as a second anode. The electron beam is aimed at the desired point on screen 16 by means of deflecting system 14 which comprises horizontal deflecting coil 20 and vertical deflecting coil 21.

Considering the operation of the illustrative system as a whole, the incoming signal is intercepted by the antenna 22 and converted to an intermediate frequency by means of the high frequency oscillator in receiver 23. The signal is usually further amplified in an intermediate fre-

quency amplifier, not shown, to a level suitable for detection. After detection, the signal is amplified in video amplifier 24 to a proper level and applied to the control grid 18 of cathode ray tube 11. This video signal is also applied to the synchronizing signal separator 25 where timing pulses are derived to synchronize the horizontal and vertical sweep generators 26 and 27. These generators supply saw-tooth waves of current to the deflection coils 20 and 21. The video signal is also applied to a color synchronizer 28 which supplies timing pulses to a high voltage switching unit 29 which in turn furnishes color signals to the post deflection electrode 30 at screen 16 to produce the proper sequence of colors.

The use of a post deflection acceleration cathode ray tube, as in the present example, is preferred because the focus and deflection of the electron beam need not be changed to correspond to each value of the high voltage applied to the screen. Of course, with the addition of proper equipment, the present system may be applied to any type of cathode ray tube as is well known to those skilled in the art.

While the present invention has been described with particular reference to a color television system, it will be appreciated that it may be applied to any equipment in which it is desired to give a precise varied color indication in a cathode ray tube. Colored radar is an example of another application of the invention.

There is provided by the present invention a multi-layer colored image producing luminescent screen which is characterized by faithful reproduction of colors at relatively low electron beam potentials and with a low voltage drop across the phosphor layers. The mono-particle thick multi-layer screen is further characterized by enhanced brightness and a minimum of internal reflection as compared to settled and other present gross or multi-particle thick layer screens. The colors produced are purer and sharper as relates to separation of one color from another. There is provided also a cathode ray tube and a television system for utilizing such a screen.

What we claim as new and desire to secure by Letters Patent of the United States is:

50. 1. A cathode ray tube screen for producing colored images comprising a plurality of uniform, mono-particle thick, continuous layers of materials producing different colored light, said layers being separated by films which absorb a part only of any electron energy passing therethrough.

60. 2. A cathode ray tube screen for producing colored images comprising a plurality of uniform, mono-particle thick layers of phosphors capable of producing different colors under cathode ray excitation, said layers being separated by films which absorb a part only of any electron energy passing therethrough.

65. 3. A cathode ray tube screen for producing colored images comprising a plurality of uniform, mono-particle thick, continuous layers of different colored light-producing material, said layers being separated by films which absorb a part only of any electron energy passing therethrough.

70. 4. A cathode ray tube screen for producing colored images comprising a plurality of uniform, mono-particle thick, continuous layers of different colored light-producing material, said layers being separated by films consisting of

silica for absorbing a portion only of any electron energy passing therethrough.

5. A cathode ray tube screen for producing colored images comprising a plurality of uniform, mono-particle thick, continuous layers of different colored light-producing material, said layers being separated by films consisting of mica for absorbing a part only of any electron energy passing therethrough.

6. A cathode ray tube screen for producing colored images comprising a plurality of uniform, mono-particle thick, continuous layers of different colored light-producing material, said layers being separated by films consisting of alkali silicate for absorbing a part only of any electron energy passing therethrough.

7. A cathode ray tube for producing colored images comprising an envelope containing electron beam producing means, means for controlling the potential of said beam, and an image screen comprising a plurality of uniform, mono-particle thick layers of phosphors capable of producing different colors under electron beam excitation, said layers being separated by films which absorb a part only of any electron energy passing therethrough.

8. A cathode ray tube for producing colored images comprising an envelope containing electron beam producing means, means for controlling the potential of said beam, and an image producing screen comprising a plurality of uniform, mono-particle thick layers of luminescent material, each layer being capable of producing a particular color under electron beam excitation, said layers being separated by films which absorb a part only of any electron energy passing therethrough.

9. A cathode ray tube for producing colored images comprising an envelope containing electron beam producing means, means for controlling the potential of said beam, and an image producing screen comprising a plurality of uniform, mono-particle thick layers of luminescent material, each layer being capable of producing a particular color under electron beam excitation, said layers being separated by films consisting of silica for absorbing a portion only of any electron energy passing therethrough.

10. A cathode ray tube for producing colored images comprising an envelope containing electron beam producing means, means for controlling the potential of said beam, and an image producing screen comprising a plurality of uniform, mono-particle thick layers of luminescent

material, each layer being capable of producing a particular color under electron beam excitation, said layers being separated by films consisting of mica for absorbing a part only of any electron energy passing therethrough.

11. A cathode ray tube for producing colored images comprising an envelope containing electron beam producing means, means for controlling the potential of said beam, and an image producing screen comprising a plurality of uniform, mono-particle thick layers of luminescent material, each layer being capable of producing a particular color under electron beam excitation, said layers being separated by films consisting of alkali silicate for absorbing a part only of any electron energy passing therethrough.

12. A color television system comprising a cathode ray tube comprising an envelope containing electron beam producing means, means for controlling the potential of said beam, and an image screen comprising a plurality of uniform, mono-particle thick layers of luminescent materials capable of producing different colors under electron beam excitation, said layers being separated by films which absorb a part only of any electron energy passing therethrough.

13. A color television system comprising a cathode ray tube comprising an envelope containing electron beam producing means, means for controlling the potential of said beam, and an image screen comprising a plurality of uniform, mono-particle thick layers of luminescent materials capable of producing different colors under electron beam excitation, said layers being separated by films which absorb a part only of any electron energy passing therethrough.

LEWIS R. KOLLER.  
FERD E. WILLIAMS.

#### REFERENCES CITED

The following references are of record in the file of this patent:

#### UNITED STATES PATENTS

| Number    | Name           | Date          |
|-----------|----------------|---------------|
| 2,343,825 | Wilson         | Mar. 7, 1944  |
| 2,423,830 | Fonda          | July 15, 1947 |
| 2,446,248 | Shrader        | Aug. 3, 1948  |
| 2,452,522 | Leverenz       | Oct. 26, 1948 |
| 2,455,710 | Szegho         | Dec. 7, 1948  |
| 2,461,515 | Bronwell       | Feb. 15, 1949 |
| 2,472,988 | Rosenthal      | June 14, 1949 |
| 2,543,477 | Sziklai et al. | Feb. 27, 1951 |
| 2,547,775 | Ramberg        | Apr. 3, 1951  |